

## UNITED STATES PATENT OFFICE

EMIL C. LOETSCHER, OF DUBUQUE, IOWA

## COMPOSITE MATERIAL AND PROCESS OF MAKING THE SAME

No Drawing.

Application filed April 17, 1929. Serial No. 355,992.

This invention relates to improvements in processes for treating cellulose materials, for the purpose of rendering the same suitable for the making of panels, doors, interior trim and like products, ordinarily fabricated of wood.

The object of the invention is to provide an improved and more economical method of treatment whereby the characteristic fibrous texture of the material acquires a surface hardness, smoothness and finish obtainable in hardwoods only by painstaking and tedious hand labor.

Inasmuch as the process is applicable for the production of various articles in which fibrous or cellulose materials are substituted for natural woods, the following description will be confined to the method of making a door panel as illustrative of the general procedure followed.

20 The base material for the panel or other piece to be made, may be any one of a number of prepared fibre or pulp boards used for insulation and wall construction, and consisting of a mass of fibres compressed into a solid sheet and having the characteristic fibrous surface texture. Having prepared a piece of the base material of proper size and thickness for a panel, the first step in its treatment is to spray on or otherwise apply to the surface, a solution of a phenol-condensation product, such as Bakelite and alcohol, although certain natural gums may be used in place of Bakelite, such as shellac, kauri or Congo gum. Bakelite is preferred as it produces a superior finish but is more costly, and therefore a cheaper substitute will often suffice, or in some cases, the Bakelite is replaced in part by one of the cheaper natural gums,—the proportion of Bakelite, however, determining the quality of the ultimate surface finish.

45 After the treatment with the Bakelite solution and while the surfaces to be finished are still partially wet and in tacky condition, a coating of pulverized or finely divided fibrous or cellulose substance, such as wood flour or ground cornstalk pulp, is sifted over the surfaces to form a coating of substantial thickness. This dry coating is then pressed 50 into the varnish-like surface by means of roll-

ers passed over the surface, or by passing the coated panel between power driven rollers, whereupon it is then subjected to a drying process in a suitable dry room or enclosure whereby the solvent remaining in the Bakelite solution is driven off, leaving the surface coating practically dry.

55 As a practical and satisfactory variation in the process, any suitable fibrous material in sheet or woven form, such as heavy paper, cardboard, or cloth, may be used in place of the pulverized substances before-mentioned. In this case, I prefer to use a thin solution of Congo gum spirit varnish dissolved in a suitable solvent, with or without the addition of varying percentages of Bakelite varnish as the primary coating for the panel surfaces. I find that Congo gum is 60 very satisfactory as an adhesive, in addition to having a high melting point, and combines readily with Bakelite, the latter being advantageous due to its hardening qualities.

65 In some respects the use of paper and the like is advantageous, in that it provides a veneer over the base material and as such materially increases the strength.

70 Continuing with the next step in the process, the dried panel is now subjected to a combined heat and pressure treatment, a press of the hydraulic type being preferably used for this purpose. Moreover, especially prepared platens or plates are provided, the same being hollow and provided with connections for the circulation of steam and cooling water therethrough for heating and cooling the platens. Depending on the degree of compactness desired in the finished panel, the pressure exerted may vary from 75 100 to 1000 pounds per square inch, it being evident that the greater the pressure the greater will be the strength of the panel. The pressure is applied for a period of from 80 five to ten minutes, during which time the platens are heated, whereupon they are allowed to cool down to the normal temperature or be artificially cooled in the manner already suggested. By reason of the application of heat, the resinous substance or 85 Bakelite, or a mixture of the two as the case 90 95 100

may be, become hardened or set, and with the accompanying pressure and cooling, a hard and smooth surface finish is produced, showing none of the characteristic fibrous 5 texture of the raw base material.

Upon removing the panel from the press, it is ready for the final surface finish. For ordinary surface decoration, paint, enamel, lacquer or varnish may be applied to the 10 panel in the same manner as they would be applied to a wood panel, although fewer coats are required due to the smooth and uniform character of the surface. If desired, the surface may be grained in imitation of natural 15 wood by any suitable graining or grain reproducing process, and a final protective coat of varnish applied, or if a more finished surface is desired, several coats of natural resin varnish or lacquer may be applied in the 20 usual manner and rubbed down, as in the case of natural wood finishes.

However, to produce what may be regarded as a fine finish, the panel may be further treated as follows: Assuming that the 25 panel has been removed from the press after the combined heat and pressure treatment, a fairly heavy solution of Bakelite varnish is applied over the surface, and the panel again placed in the drying room for the purpose of 30 expelling the solvent in the Bakelite varnish solution. At first, the drying is allowed to continue slowly at a relatively low temperature, which is gradually increased to from 240° to 280° F., at which temperatures the 35 solvent is driven off and the Bakelite changed from a soluble fusible state to an insoluble and partially infusible state, that is to say, short of its final state of infusibility, as that 40 would render it incapable of further treatment. But with the Bakelite coating still fusible in some degree after the drying process, the panel is again placed in the press and subjected to pressure of from 100 to 1000 pounds per square inch, depending on 45 the desired strength of the panel. As before, the press is equipped with hollow platens into which steam is admitted.

In this manner, the Bakelite coating is 50 subjected to a temperature of say 250° F. to 275° F. for a period sufficient to cure the Bakelite. Ordinarily, one-half hour at the 55 temperature stated is adequate, although the time may be shortened by increasing the temperature.

During the heating process in the press, the Bakelite first becomes fusible and spreads 60 over the surface of the panel in a smooth, even film, and later becomes infusible. When this condition is reached, the platens are then cooled by water, and the panel removed from the press.

This final treatment with Bakelite varnish 65 produces an exceptionally high grade finish and one capable of withstanding hard wear and usage, and injury by contact with ordi-

nary acids and solvents, or exposure to temperatures as high as 400° F.

As will be seen from the foregoing, the process may be carried only to the point of producing finishes suitable for ordinary interior work, or may continue to the point of providing an exceedingly hard and lasting surface, having all of the lustre and beauty obtainable in natural woods, but of greater desirability and at a greatly reduced cost, 70 both as to the raw materials and the labor involved.

Having set forth a preferred embodiment of my invention, I claim as new and novel:

1. A process for producing a composite 80 material consisting of coating a sheet of base material composed of a partially compressed mass of cellulosic fiber pulp with a resinous varnish and drying the same to provide a tacky surface, applying a thin layer of pulverized fibrous material over said surface, subjecting said base sheet to heat and pressure, applying a solution of a phenol-condensate product over the surface of the treated sheet and again subjecting the same to heat sufficient to render said product hard and infusible. 85

2. A process for producing a composite 90 material consisting of coating a sheet of fibrous material derived from corn-stalk or wood pulp with a resinous varnish, applying a thin layer of fibrous material over said coated surface, subjecting said base sheet to heat and pressure treatment, applying a phenol-condensate product over the surface 95 of the treated sheet and again subjecting the same to heat sufficient to render said product hard and infusible. 100

Signed at Dubuque this 12 day of April, 1929. 105

EMIL C. LOETSCHER.

110

115

120

125

130